



US006265145B1

(12) **United States Patent**  
Mehta et al.

(10) **Patent No.:** US 6,265,145 B1  
(45) **Date of Patent:** Jul. 24, 2001

(54) **PROCESS FOR THE PREPARATION OF HIGH CHLORIDE EMULSIONS CONTAINING IODIDE**

(75) Inventors: **Rajesh V. Mehta**, Rochester; **Jerzy A. Budz**, Fairport; **Jess B. Hendricks, III**, Rochester; **Heinz E. Stapelfeldt**; **Seshadri Jagannathan**, both of Pittsford; **Ramesh Jagannathan**, Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/475,405**

(22) Filed: **Dec. 30, 1999**

**Related U.S. Application Data**

(63) Continuation-in-part of application No. 09/218,683, filed on Dec. 22, 1998, now Pat. No. 6,048,683.

(51) **Int. Cl.<sup>7</sup>** ..... **G03C 1/005**; G03C 1/035

(52) **U.S. Cl.** ..... **430/569**; 430/567

(58) **Field of Search** ..... 430/567, 569

(56) **References Cited**

**U.S. PATENT DOCUMENTS**

|             |         |                              |
|-------------|---------|------------------------------|
| 4,539,290   | 9/1985  | Mumaw .                      |
| 4,865,962   | 9/1989  | Hasebe et al. .              |
| 5,252,454   | 10/1993 | Suzumoto et al. .            |
| 5,252,456   | 10/1993 | Ohshima et al. .             |
| 5,547,827   | 8/1996  | Chen et al. .                |
| 5,549,879   | 8/1996  | Chow .                       |
| 5,550,013   | 8/1996  | Chen et al. .                |
| 5,605,789   | 2/1997  | Chen et al. .                |
| 5,726,005   | 3/1998  | Chen et al. .                |
| 5,728,516   | 3/1998  | Edwards et al. .             |
| 5,736,310   | 4/1998  | Chen et al. .                |
| 5,750,327   | 5/1998  | Chang et al. .               |
| 5,783,372   | 7/1998  | Budz et al. .                |
| 5,783,373   | 7/1998  | Mydlarz et al. .             |
| 5,783,378   | 7/1998  | Mydlarz et al. .             |
| 5,792,601 * | 8/1998  | Edwards et al. ..... 430/567 |
| 6,030,762 * | 2/2000  | Verrept et al. .             |
| 6,048,683   | 4/2000  | Mehta et al. .               |

**OTHER PUBLICATIONS**

Research Disclosure, "Mixer for Improved Control Over Reaction Environment", 38213, Feb. 1996, pp. 111-114.

Research Disclosure, "Photographic Silver Halide Emulsions, Preparations, Addenda, Systems And Processing", 38957 (I), Sep. 1996, pp. 591-598.

Research Disclosure, "A Robust Method For The Preparation Of High Chloride Emulsions", 41955, Mar. 1999, pp. 345-350.

\* cited by examiner

*Primary Examiner*—Janet Baxter

*Assistant Examiner*—Amanda C. Walke

(74) *Attorney, Agent, or Firm*—Andrew J. Anderson

(57) **ABSTRACT**

A process for the preparation of a radiation-sensitive silver halide emulsion comprised of high chloride cubical silver halide grains containing from 0.05 to 3 mole percent iodide, based on total silver, where the iodide is incorporated in the grains in a controlled, non-uniform distribution forming a core containing at least 50 percent of total silver, an iodide free surface shell having a thickness of greater than 50 Å, and a sub-surface shell that contains a maximum iodide concentration is disclosed, the process comprising: (a) providing in a stirred reaction vessel a dispersing medium and host high chloride silver halide cubical grains comprising a speed enhancing amount of iodide, and (b) precipitating silver halide onto the host grains by introducing at least a silver salt solution into the dispersing medium at a rate such that the normalized molar addition rate,  $R_n$ , is above  $3.0 \times 10^{-2} \text{ min}^{-1}$ ,  $R_n$  satisfying the formula:

$$R_n = [Q_f \times C_f] / M$$

where  $Q_f$  is the volumetric rate of addition, in L/min, of silver salt solution into the reaction vessel;  $C_f$  is the concentration, in moles/L, of the silver salt solution; and  $M$  is total moles of silver halide in the host grains in the reaction vessel at the precise moment of addition of the silver salt solution. In a further aspect, this invention is directed towards a photographic recording element comprising a support and at least one light sensitive silver halide emulsion layer comprising silver halide grains prepared as described above. The advantages of the invention are generally accomplished in accordance with the discovery that when the exterior portion of profiled silver iodochloride grains are grown under specific conditions of high molar addition rates, iodochloride emulsions of enhanced sensitivity and photographic curve shape are produced, as speed can be increased while keeping fog to a low level.

**17 Claims, No Drawings**

**PROCESS FOR THE PREPARATION OF  
HIGH CHLORIDE EMULSIONS  
CONTAINING IODIDE**

**CROSS-REFERENCE TO RELATED  
APPLICATIONS**

This application is a continuation-in-part of commonly assigned U.S. Ser. No. 09/218,683, filed Dec. 22, 1998, now U.S. Pat. No. 6,048,683, the disclosure of which is incorporated by reference herein.

**FIELD OF THE INVENTION**

This invention is directed to the preparation of radiation sensitive silver iodochloride emulsions useful in photography, including electronic printing methods wherein information is recorded in a pixel-by-pixel mode in a radiation sensitive silver halide emulsion layer. It particularly relates to the preparation of the exterior portions of emulsion grains after formation of a maximum iodide concentration sub-surface shell surrounding a central portion.

**DEFINITION OF TERMS**

The term "high chloride" in referring to silver halide grains and emulsions indicates that chloride is present in a concentration of greater than 50 mole percent, based on total silver.

In referring to grains and emulsions containing two or more halides, the halides are named in order of ascending concentrations.

The term "cubic grain" is employed to indicate a grain is that bounded by six {100} crystal faces. Typically the corners and edges of the grains show some rounding due to ripening, but no identifiable crystal faces other than the six {100} crystal faces. The six {100} crystal faces form three pairs of parallel {100} crystal faces that are equidistantly spaced.

The term "cubical grain" is employed to indicate grains that are at least in part bounded by {100} crystal faces satisfying the relative orientation and spacing of cubic grains. That is, three pairs of parallel {100} crystal faces are equidistantly spaced. Cubical grains include both cubic grains and grains that have one or more additional identifiable crystal faces. For example, tetradecahedral grains having six {100} and eight {111} crystal faces are a common form of cubical grains.

The term "central portion" in referring to cubical silver halide grains refers to that portion of the grain structure that is first precipitated accounting for up to 98 percent of total precipitated silver required to form the {100} crystal faces of the grains.

The term "dopant" is employed to indicate any material within the rock salt face centered cubic crystal lattice structure of a silver halide grain other than silver ion or halide ion.

The term "dopant band" is employed to indicate the portion of the grain formed during the time that dopant was introduced to the grain during precipitation process.

The term "normalized" molar addition rate hereinafter assigned the symbol  $R_n$  is a measure of the intensity of rate of addition of silver salt solution to the reaction vessel in case of a double-jet precipitation process.  $R_n$  is defined by the formula:

$$R_n = Q_f C_f M$$

where  $Q_f$  is the volumetric rate (liters/min) of addition of silver salt solution into the reaction vessel,  $C_f$  is the molar

concentration (moles/liter) of the said solution, and  $M$  is total moles of silver halide host grains in the reaction vessel at the precise moment of above addition.

All references to the periodic table of elements periods 5 and groups in discussing elements are based on the Periodic Table of Elements as adopted by the American Chemical Society and published in the *Chemical and Engineering News*, Feb. 4, 1985, p. 26. The term "Group VIII" is used to generically describe elements in groups 8, 9 and 10.

10 The term "log E" is the logarithm of exposure in lux-seconds.

Photographic speed is reported in relative log units and therefore referred to as relative log speed. 1.0 relative log speed unit is equal to 0.01 log E.

15 The term "contrast" or "γ" is employed to indicate the slope of a line drawn from stated density points on the characteristic curve.

The term "reciprocity law failure" refers to the variation in response of an emulsion to a fixed light exposure due to 20 variation in the specific exposure time.

*Research Disclosure* is published by Kenneth Mason Publications, Ltd., Dudley House, 12 North St., Emsworth, Hampshire PO10 7DQ, England.

**BACKGROUND**

25 In its most commonly practiced form silver halide photography employs a film in a camera to produce, following photographic processing, a negative image on a transparent film support. A positive image for viewing is produced by 30 exposing a photographic print element containing one or more silver halide emulsion layers coated on a reflective white support through the negative image in the camera film, followed by photographic processing. In a relatively recent variation negative image information is retrieved by scanning and stored in digital form. The digital image information is later used to expose imagewise the emulsion layer or 35 layers of the photographic print element.

Whereas high bromide silver halide emulsions are the overwhelming commercial choice for camera films, high 40 chloride cubic grain emulsions are the overwhelming commercial choice for photographic print elements. It is desired in high chloride emulsions for color paper applications to obtain high photographic speed at the desired curve shape. While it has been common practice to avoid or minimize the

45 incorporation of iodide into high chloride grains employed in color paper, it has been recently observed that silver iodochloride cubical grains can offer exceptional levels of photographic speed where iodide is incorporated in such emulsion gains in a profiled manner. Chen et. al. in U.S. Pat.

50 No. 5,547,827; Chen et. al. in U.S. Pat. No. 5,550,013; Chen et. al. in U.S. Pat. No. 5,605,789; Chen et. al. in U.S. Pat. No. 5,726,005; Edwards et.al. in U.S. Pat. No. 5,728,516; Chen et. al. in U.S. Pat. No. 5,736,310; Budz et.al. in U.S. Pat. No. 5,783,372 and Edwards et.al. in U.S. Pat. No. 5,792,601

55 disclose highly sensitive silver iodochloride cubical emulsions with low levels of iodide located in the exterior portions of the grains. The interior portions of such grains can be prepared by employing any convenient high chloride cubical grain precipitation procedure. The emulsion grains

60 thus formed then serve as hosts for further growth. Once a host grain population has been prepared, an increased concentration of iodide is introduced into the emulsion to form the region of the grains containing maximum iodide concentration. The source of iodide ion can be silver iodide

65 grains or any iodide-releasing agent, but it is typically disclosed that iodide is preferably introduced alone as an aqueous solution of an alkali metal iodide salt. This is

followed by double-jet introduction of silver nitrate and alkali metal chloride solutions at conventional molar addition rates, constant or ramped, till the exterior portion is grown to the desired size.

Chow U.S. Pat. No. 5,549,879 discloses a pulsed flow double jet technique for preparing silver halide grains. Chow discloses introducing an aqueous silver nitrate solution from a remote source by a conduit which terminates close to an adjacent inlet zone of a mixing device, which is disclosed in greater detail in *Research Disclosure*, Vol. 382, February 1996, Item 38213. Simultaneously with the introduction of the aqueous silver nitrate solution and in an opposing direction, aqueous halide solution is introduced from a remote source by a conduit which terminates close to an adjacent inlet zone of the mixing device. The mixing device is vertically disposed in a reaction vessel and attached to the end of a shaft, driven at high speed by any suitable means. The lower end of the rotating mixing device is spaced up from the bottom of the vessel, but beneath the surface of the aqueous silver halide emulsion contained within the vessel. Baffles, sufficient in number to inhibit horizontal rotation of the contents of the vessel are located around the mixing device.

Chow teaches operating the described apparatus in a "pulse flow" manner comprising the steps of: (a) providing an aqueous solution containing silver halide particles having a first grain size; (b) continuously mixing the aqueous solution containing silver halide particles; (c) simultaneously introducing a soluble silver salt solution and a soluble halide salt solution into a reaction vessel of high velocity turbulent flow confined within the aqueous solution for a time  $t$ , wherein  $t$  is at least 1000 rpm; (d) simultaneously halting the introduction of the soluble silver salt solution and the soluble halide salt solution into the reaction for a time  $T$  wherein  $T > t$ , thereby allowing the silver halide particles to grow; and (e) repeating steps (c) and (d) until the silver halide particles attain a second grain size greater than the first grain size. Chow teaches the pulse flow technique to permit easier scalability of the precipitation method. There is no disclosure of use of such pulse flow technique to prepare profiled silver iodochloride emulsion grains.

#### PROBLEM TO BE SOLVED BY THE INVENTION

There is continuing need for iodochloride emulsions with enhanced photographic sensitivity while controlling the toe region of the photographic response curve at the minimum fog level. The enhanced sensitivity emulsions would be useful to build specific photographic elements for detailed tone scale differentiation. Increased emulsion photographic sensitivity, however, often results in difficulties in emulsion manufacturing. These difficulties manifest themselves as sensitivity of the photographic response to the reactor hydrodynamic condition during precipitation, as controlled by the level of agitation.

One objective of the present invention accordingly is to provide silver iodochloride emulsions with enhanced sensitivity.

A further objective is to provide color papers that have improved tonal scale at the toe region of the photographic curve.

A still further objective is to improve the process of silver iodochloride emulsion manufacturing.

#### SUMMARY OF THE INVENTION

In one aspect this invention is directed towards a process for the preparation of a radiation-sensitive silver halide

emulsion comprised of high chloride cubical silver halide grains containing from 0.05 to 3 mole percent iodide, based on total silver, where the iodide is incorporated in the grains in a controlled, non-uniform distribution forming a core containing at least 50 percent of total silver, an iodide free surface shell having a thickness of greater than 50 Å, and a sub-surface shell that contains a maximum iodide concentration, the process comprising: (a) providing in a stirred reaction vessel a dispersing medium and host high chloride silver halide cubical grains comprising a speed enhancing amount of iodide, and (b) precipitating silver halide onto the host grains by introducing at least a silver salt solution into the dispersing medium at a rate such that the normalized molar addition rate,  $R_n$ , is above  $3.0 \times 10^{-2} \text{ min}^{-1}$ ,  $R_n$  satisfying the formula:

$$R_n = [Q_f \times C_f] / M$$

where  $Q_f$  is the volumetric rate of addition, in L/min, of silver salt solution into the reaction vessel;  $C_f$  is the concentration, in moles/L, of the silver salt solution; and  $M$  is total moles of silver halide in the host grains in the reaction vessel at the precise moment of addition of the silver salt solution.

In a further aspect, this invention is directed towards a photographic recording element comprising a support and at least one light sensitive silver halide emulsion layer comprising silver halide grains prepared as described above.

The advantages of the invention are generally accomplished in accordance with the discovery that when the exterior portion of profiled silver iodochloride grains are grown under specific conditions of high molar addition rates, iodochloride emulsions of enhanced sensitivity and photographic curve shape are produced, as speed can be increased while keeping fog to a low level.

#### DESCRIPTION OF PREFERRED EMBODIMENTS

The cubical silver halide grains precipitated in accordance with the invention contain greater than 50 mole percent chloride, based on silver. Preferably the grains contain at least 70 mole percent chloride and, optimally at least 90 mole percent chloride, based on silver. Overall iodide concentration is from 0.05 to 3 mole percent, preferably 0.1 to 1 mole percent, based on silver. Silver bromide and silver chloride are miscible in all proportions. Hence, any portion of the total halide not accounted for chloride and iodide, can be bromide. For color reflection print (i.e., color paper) uses bromide is typically limited to less than 10 mole percent based on silver and iodide is preferably limited to less than 1 mole percent based on silver.

It has been recognized for the first time that heretofore unattained levels of sensitivity and other advantageous properties, such as those recited in the objects and demonstrated in the samples below, can be realized, without offsetting degradation of photographic performance, by the controlled, non-uniformly distributed incorporation of iodide within the grains using a process of this invention. Specifically, after at least 50 (preferably 85) percent of total silver forming the grains has been precipitated to form a core or central portion of the grains, a maximum iodide concentration is located within a shell that is formed on the host (core) grains, and the maximum iodide concentration containing shell is then converted to a sub-surface shell by precipitating silver and halide ions without further iodide addition, where the exterior portion of the grain surround the central core portion is grown under high normalized molar addition rates,  $R_n$ .

In accordance with the emulsions of the invention, iodide addition onto core portions of the grains creates a silver iodochloride shell on the host (core) high chloride grains. Attempts to use these shelled grains in photographic print elements without further modification results in markedly inferior performance. Having high iodide concentrations at the surface of the grains lowers speed as compared to the emulsions satisfying the requirements of the invention when both emulsions are sensitized to the same minimum density and otherwise produces elevated levels of minimum density that are incompatible with acceptable performance characteristics of photographic reflective print elements.

To increase speed and lower minimum density an iodide-free shell is precipitated onto the silver iodochloride shell, converting it into a sub-surface shell. The depth to which sub-surface shell is buried is chosen to render the iodide in the sub-surface shell inaccessible to the developing agent at the outset of development of latent image bearing grains and inaccessible throughout development in the grains that do not contain a latent image. The thickness of the surface shell is contemplated to be greater than 50 Å in emulsions employed in reflection print photographic elements. The surface shell thickness can, of course, range up to any level compatible with the minimum core requirement of 50 (preferably 85) percent of total silver. Since the sub-surface shell can contribute as little as 0.05 mole percent iodide, based on total silver, it is apparent that surface shells can account for only slightly less than all of the silver not provided by the core portions of the grains. A surface shell accounting for just less than 50 (preferably just less than 15) percent of total silver is specifically contemplated. Whereas it might be thought that shifting the maximum iodide phase to the interior of the grain would also shift the latent image internally, detailed investigations have revealed that latent image formation remains at the surface of the grains. It is surprising that burying the maximum iodide phase within the grains using high rates of reagents addition not only is compatible with achieving higher levels of photoefficiency but actually contributes an additional increment of speed enhancement.

It was initially observed that, after starting with monodisperse silver chloride cubic grains (i.e., grains consisting of six {100} crystal faces), iodide introduction produced tetradecahedral grains (i.e., grains consisting of six {100} crystal faces and eight {111} crystal faces). Further investigations revealed that as few as one {111} crystal face are sometimes present in the completed grains. On still further investigation, it has been observed that the emulsions of the invention can be cubic grain emulsions. Thus, although the presence of at least {111} crystal face (and usually tetradecahedral grains), provides a convenient visual clue that the grains may have been prepared according to the teaching of this invention, it has now been concluded that one or more {111} crystal faces are a by-product of grain formation that can be eliminated or absent without compromising the unexpected performance advantages of the invention noted above.

The preparation of cubical grain silver iodochloride emulsions with iodide placements that produce increased photographic sensitivity can be undertaken by employing any convenient conventional high chloride cubical grain precipitation procedure prior to precipitating the region of maximum iodide concentration—that is, through the introduction of at least the first 50 (preferably at least the first 85) percent of silver precipitation. The initially formed high chloride cubical grains then serve as hosts for further grain growth. In one specifically contemplated preferred form the host

emulsion is a monodisperse silver chloride cubic grain emulsion. Low levels of iodide and/or bromide, consistent with the overall composition requirements of the grains, can also be tolerated within the host grains. The host grains can include other cubical forms, such as tetradecahedral forms. Techniques for forming emulsions satisfying the host grain requirements of the preparation process are well known in the art. For example, prior to growth of the maximum iodide concentration region of the grains, the precipitation procedures of Atwell U.S. Pat. No. 4,269,927, Tanaka EPO 0 080 10 905, Hasebe et al U.S. Pat. No. 4,865,962, Asami EPO 0 295 439, Suzumoto et al U.S. Pat. No. 5,252,454 or Ohshima et al U.S. Pat. No. 5,252,456, the disclosures of which are here incorporated by reference, can be employed, but with those portions of the preparation procedures, when present, that place bromide ion at or near the surface of the grains being omitted. Stated another way, the host grains can be prepared employing the precipitation procedures taught by the citations above through the precipitation of the highest chloride concentration regions of the grains they prepare. The rate at which silver nitrate and sodium chloride are added into the reactor during precipitation of the host grains can be at any practical normalized molar addition rate range, including low ( $R_n$  less than or equal to  $0.03 \text{ min}^{-1}$ ) and high ( $R_n$  greater than  $0.03 \text{ min}^{-1}$ ) addition rates.

Once a host grain population has been prepared accounting for at least 50 percent (preferably at least 85 percent) of total silver has been precipitated, an increased concentration of iodide is introduced into the emulsion to form the region of the grains containing a maximum iodide concentration. The iodide ion is preferably introduced as a soluble salt, such as an ammonium or alkali metal iodide salt. The iodide ion can be introduced concurrently with the addition of silver and/or chloride ion. Alternatively, the iodide ion can be introduced alone followed promptly by silver ion introduction with or without further chloride ion introduction. As an alternative source of iodide ions, the fine silver iodide grains of a Lippmann emulsion can be ripened out as disclosed anonymously in *Research Disclosure*, Vol. 531, 30 May 1998, item 40928. Still another approach, recently 35 advocated, illustrated by Royster et al in U.S. Pat. No. 5,866,314, is to add iodide as dimethylamine silver chloro-iodide complex. It is preferred to grow the maximum iodide concentration region on the surface of the host grains rather than to introduce a maximum iodide concentration region 40 exclusively by displacing chloride ion adjacent the surfaces of the host grains.

To maximize the localization of crystal lattice variances produced by iodide incorporation it is preferred that the iodide ion be introduced as rapidly as possible. That is, the iodide ion forming the maximum iodide concentration region of the grains is preferably introduced in less than 30 seconds, optimally in less than 10 seconds. When the iodide is introduced more slowly, somewhat higher amounts of iodide (but still within the ranges set out above) are required to achieve speed increases equal to those obtained by more rapid iodide introduction and minimum density levels are somewhat higher. Slower iodide additions are manipulatively simpler to accomplish, particularly in larger batch size emulsion preparations. Hence, adding iodide over a period of at least 1 minute (preferably at least 2 minutes) and, 50 preferably, during the concurrent introduction of silver is specifically contemplated.

After the iodide addition, silver salt solution is added add a high normalized molar addition rate (i.e.,  $R_n$  greater than  $0.03 \text{ min}^{-1}$ , preferably greater than or equal to  $0.05 \text{ min}^{-1}$ ) in accordance with the invention to create an outer shell. Where the reaction vessel contains excess halide ions, the

silver salt solution may be added by itself to precipitated the outer shell. It is preferred, however, to simultaneously introduce a halide salt solution into the dispersing medium with the silver salt solution. It is surprising that burying the maximum iodide phase within the grains using high rates of reagents addition not only is compatible with achieving higher levels of photoefficiency but actually contributes an additional increment of speed enhancement.

At the conclusion of grain precipitation the grains can take varied cubical forms, ranging from cubic grains (bounded entirely by six {100} crystal faces), grains having an occasional identifiable {111} face in addition to six {100} crystal faces, and, at the opposite extreme tetradecahedral grains having six {00} and eight {111} crystal faces.

After examining the performance of emulsions exhibiting varied cubical grain shapes, it has been concluded that the performance of these emulsions is principally determined by iodide incorporation and the uniformity of grain size dispersity. The silver iodochloride grains are relatively mono-disperse. The silver iodochloride grains preferably exhibit a grain size coefficient of variation of less than 35 percent and optimally less than 25 percent. Much lower grain size coefficients of variation can be realized, but progressively smaller incremental advantages are realized as dispersity is minimized.

It is specifically contemplated to incorporate dopants into the silver halide emulsion grains of the invention during precipitation. The use of dopants in silver halide grains to modify photographic performance is generally illustrated by *Research Disclosure*, Item 38957, cited above, I. Emulsion grains and their preparation, D. Grain modifying conditions and adjustments, paragraphs (3)–(5).

Photographic performance attributes known to be affected by dopants include sensitivity, reciprocity failure, and contrast.

In accordance with preferred embodiments of the invention, iridium coordination complex dopants may be incorporated into the face centered cubic crystal lattice of the emulsion grains. The iridium coordination complex dopant preferably is an iridium coordination complex having ligands each of which are more electropositive than a cyano ligand. The iridium dopant preferably contains at least one thiazole or substituted thiazole ligand. The thiazole ligands may be substituted with any photographically acceptable substituent which does not prevent incorporation of the dopant into the silver halide grain. Exemplary substituents include lower alkyl (e.g., alkyl groups containing 1–4 carbon atoms), and specifically methyl. A specific example of a substituted thiazole ligand which may be used in accordance with the invention is 5-methylthiazole. In a specifically preferred form the remaining non-thiazole or non-substituted-thiazole ligands of the iridium coordination complexe dopants are halide ligands. It is specifically contemplated to select iridium coordination complex dopants from among the coordination complexes containing organic ligands disclosed by Olm et al U.S. Pat. No. 5,360,712, Olm et al U.S. Pat. No. 5,457,021 and Kuromoto et al U.S. Pat. No. 5,462,849, the disclosures of which are here incorporated by reference.

In a preferred form it is contemplated to employ as the iridium dopant a hexacoordination complex satisfying the formula:



wherein

$n$  is zero, -1, -2, -3 or -4; and

$\text{L}_6$  represents six bridging ligands which can be independently selected, provided that at least four of the ligands are anionic ligands. Preferably, each of the ligands is more

electropositive than a cyano ligand, and at least one of the ligands comprises a thiazole or substituted thiazole ligand. Any remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. In a specifically preferred form at least four of the ligands are halide ligands, such as chloride or bromide ligands. Useful neutral and anionic organic ligands for dopant hexacoordination complexes are also disclosed by Olm et al U.S. Pat. No. 5,360,712 and Kuromoto et al U.S. Pat. No. 5,462,849, the disclosures of which are here incorporated by reference.

When the iridium coordination complex dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated.

The following are specific illustrations of dopants capable of use in the invention:



The iridium dopants are effective at some level at any location within the grains. Generally better results are obtained when the dopant is incorporated in the exterior 50 percent of the grain, based on silver. To insure that the dopant is in fact incorporated in the grain structure and not merely associated with the surface of the grain, it is possible to introduce the dopant prior to forming, during or after forming the maximum iodide concentration region of the grain. In accordance with a preferred embodiment, however, an iridium dopant may be introduced prior to formation of the high iodide band (within a region adjacent to the high iodide band and comprising up 60% of the total silver into the emulsion grains, preferably up to 40% of the total silver, and most preferably up to 20% of the total silver), or incorporated into the high iodide band by introducing the dopant into the reaction vessel as a single-jet with iodide solution, as disclosed in concurrently filed, copending, commonly assigned U.S. Ser. No. 09/475,841 (Kodak Docket No. 80209AJA), the disclosure of which is incorporated by reference herein. Generally better results are obtained when the dopant is incorporated in the exterior 50 percent of the grain, based on silver. Thus, an optimum grain region for dopant incorporation is that formed by silver ranging from 0 to 50 percent of total silver prior to iodide addition. That is, dopant introduction is optimally commenced after 50 percent minus the shell volume over iodide band of total silver has been introduced. The dopant can be introduced all at once or run into the reaction vessel over a period of time while grain precipitation is continuing. It is preferred to run dopant over a period of time, thus forming a dopant band within the grain.

The iridium dopants can be employed in any conventional useful concentration, and are generally used in an amount between  $1\times10^{-10}$  and  $1\times10^{-5}$  moles per silver mole. A preferred amount of the iridium is between  $1\times10^{-9}$  and  $1\times10^{-6}$  moles per silver mole for best photographic performance.

The contrast of photographic elements containing silver iodochloride emulsions of the invention can be further increased by doping the silver iodochloride grains with a hexacoordination complex containing a nitrosyl or thionitrosyl ligand. Preferred coordination complexes of this type are represented by the formula:



where

T is a Os or Ru;

E is a bridging ligand;

E' is E or NZ;

r is zero, -1, -2 or -3; and

Z is oxygen or sulfur.

The E ligands can take any of the forms found in the dopants. A listing of suitable coordination complexes satisfying the above formula is found in McDugle et al U.S. Pat. No. 4,933,272, the disclosure of which is here incorporated by reference.

Osmium and ruthenium dopants such as described in U.S. Pat. No. 5,830,631, the disclosure of which is hereby incorporated by reference, may also be used in the emulsions of the invention.

The emulsions can be prepared in any mean grain size known to be useful in photographic print elements. Mean grain sizes in the range of from 0.15 to 2.5  $\mu\text{m}$  are typical, with mean grain sizes in the range of from 0.2 to 2.0  $\mu\text{m}$  being generally preferred.

Once high chloride cubical grains having profiled iodide concentration have been precipitated as described above, chemical and spectral sensitization, followed by the addition of conventional addenda to adapt the emulsion for the imaging application of choice can take any convenient conventional form. These conventional features are illustrated by *Research Disclosure*, Item 38957, cited above, particularly:

III. Emulsion washing;

IV. Chemical sensitization;

V. Spectral sensitization and desensitization;

VII. Antifoggants and stabilizers;

VIII. Absorbing and scattering materials;

IX. Coating and physical property modifying addenda; and

X. Dye image formers and modifiers.

Some additional silver halide, generally less than 5 percent and typically less than 1 percent, based on total silver, can be introduced to facilitate chemical sensitization. It is also recognized that silver halide can be epitaxially deposited at selected sites on a host grain to increase its sensitivity. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains

while silver halide that deposits and provides the final {100} crystal faces of the grains is included in the total silver forming the grains, even when it differs significantly in composition from the previously precipitated silver halide.

The emulsions of the invention may be chemically sensitized as known in the art. Preferred chemical sensitizers include gold and sulfur chemical sensitizers. Typical of suitable gold and sulfur sensitizers are those set forth in Section IV of *Research Disclosure* 38957, September 1996. Preferred is colloid aurous sulfide such as disclosed in *Research Disclosure* 37154 for good speed and low fog.

It is also possible to add dopants during emulsion finishing. It is preferred in the invention that an iridium complex additionally be added during finishing in order to produce a print material with good reciprocity performance. The preferred iridium complex for addition during finishing is an iridium hexachloride compound, which is preferably added in an amount between 0.0001 and 1.0 mg/silver mole, more preferably between 0.001 and 0.1 mg/silver mole, for best photographic performance. It is specifically contemplated to add additional iridium dopants to the emulsions of the invention during finishing with epitaxially deposited silver bromide after the iodide sub-surface shell has been formed by the addition of AgI seeds as described in copending, concurrently filed U.S. Ser. No. 09/475,839 (Kodak Docket 80208AJA) of Budz et al., the disclosure of which is incorporated by reference herein.

The emulsions can be spectrally sensitized in any convenient conventional manner. Spectral sensitization and the selection of spectral sensitizing dyes is disclosed, for example, in *Research Disclosure*, Item 38957, cited above, Section V. Spectral sensitization and desensitization. The emulsions used in the invention can be spectrally sensitized with dyes from a variety of classes, including the polymethine dye class, which includes the cyanines, merocyanines, complex cyanines and merocyanines (i.e., tri-, tetra- and polynuclear cyanines and merocyanines), styryls, merostyryls, streptocyanines, hemicyanines, arylidenes, allopolar cyanines and enamine cyanines. Combinations of spectral sensitizing dyes can be used which result in supersensitization—that is, spectral sensitization greater in some spectral region than that from any concentration of one of the dyes alone or that which would result from the additive effect of the dyes. Supersensitization can be achieved with selected combinations of spectral sensitizing dyes and other addenda such as stabilizers and antifoggants, development accelerators or inhibitors, coating aids, brighteners and antistatic agents. Any one of several mechanisms, as well as compounds which can be responsible for supersensitization, are discussed by Gilman, *Photographic Science and Engineering*, Vol.18, 1974, pp. 418-430.

The silver iodochloride emulsions are preferably protected against changes in fog upon aging. Preferred antifoggants can be selected from among the following groups:

A. A mercapto heterocyclic nitrogen compound containing a mercapto group bonded to a carbon atom which is linked to an adjacent nitrogen atom in a heterocyclic ring system,

B. A quaternary aromatic chalcogenazolium salt wherein the chalcogen is sulfur, selenium or tellurium,

C. A triazole or tetrazole containing an ionizable hydrogen bonded to a nitrogen atom in a heterocyclic ring system, or

D. A dichalcogenide compound comprising an —X—X— linkage between carbon atoms wherein each X is divalent sulfur, selenium or tellurium.

The above groups of antifoggants are known in the art, and are described in more detail, e.g., in U.S. Ser. No. 5,792,601, the disclosure of which is incorporated by reference herein.

In the simplest contemplated form a recording element in accordance with the invention can consist of a single emulsion layer satisfying the emulsion description provided above coated on a conventional photographic support, such as those described in *Research Disclosure*, Item 38957, cited above, XVI. Supports. In one preferred form the support is a white reflective support, such as photographic paper support or a film support that contains or bears a coating of a reflective pigment. To permit a print image to be viewed using an illuminant placed behind the support, it is preferred to employ a white translucent support, such as a Duratrans™ or Duraclear™ support.

The invention can be used to form either silver or dye images in the recording element. In a simple form a single radiation sensitive emulsion layer unit is coated on the support. The emulsion layer unit can contain one or more high chloride silver halide emulsions satisfying the requirements of the invention, either blended or located in separate layers. When a dye imaging forming compound, such as a dye-forming coupler, is present in the layer unit, it can be present in an emulsion layer or in a layer coated in contact with the emulsion layer. With a single emulsion layer unit a monochromatic image is obtained.

It is, of course, recognized that the photographic elements of the invention can include more than one emulsion. Where more than one emulsion is employed, such as in a photographic element containing a blended emulsion layer or separate emulsion layer units, all of the emulsions can be silver iodochloride emulsions as contemplated by this invention. Alternatively one or more conventional emulsions can be employed in combination with the silver iodochloride emulsions of this invention. For example, a separate emulsion, such as a silver chloride or bromochloride emulsion, can be blended with a silver iodochloride emulsion according to the invention to satisfy specific imaging requirements. For example, emulsions of differing speed are conventionally blended to attain specific aim photographic characteristics. Instead of blending emulsions, the same effect can usually be obtained by coating the emulsions that might be blended in separate layers. It is well known in the art that increased photographic speed can be realized when faster and slower emulsions are coated in separate layers with the faster emulsion layer positioned to receiving exposing radiation first. When the slower emulsion layer is coated to receive exposing radiation first, the result is a higher contrast image. Specific illustrations are provided by *Research Disclosure*, Item 36544, cited above Section I. Emulsion grains and their preparation, Subsection E. Blends, layers and performance categories.

The emulsion layers as well as optional additional layers, such as overcoats and interlayers, contain processing solution permeable vehicles and vehicle modifying addenda. Typically these layer or layers contain a hydrophilic colloid, such as gelatin or a gelatin derivative, modified by the addition of a hardener. Illustrations of these types of materials are contained in *Research Disclosure*, Item 36544, previously cited, Section II. Vehicles, vehicle extenders, vehicle-like addenda and vehicle related addenda. The overcoat and other layers of the photographic element can usefully include an ultraviolet absorber, as illustrated by *Research Disclosure*, Item 36544, Section VI. UV dyes/optical brighteners/luminescent dyes, paragraph (1). The overcoat, when present can usefully contain matting agents to reduce surface adhesion. Surfactants are commonly added to the coated layers to facilitate coating. Plasticizers and lubricants are commonly added to facilitate the physical handling properties of the photographic elements. Antistatic

agents are commonly added to reduce electrostatic discharge. Illustrations of surfactants, plasticizers, lubricants and matting agents are contained in *Research Disclosure*, Item 36544, previously cited, Section IX. Coating physical property modifying addenda.

Preferably the photographic elements of the invention include a conventional processing solution decolorizable antihalation layer, either coated between the emulsion layer(s) and the support or on the back side of the support. Such layers are illustrated by *Research Disclosure*, Item 36544, cited above, Section VIII. Absorbing and Scattering Materials, Subsection B, Absorbing materials and Subsection C. Discharge.

A specific preferred application of the invention is in color photographic elements, particularly color print (e.g., color paper) photographic elements intended to form multicolor images. In multicolor image forming photographic elements at least three superimposed emulsion layer units are coated on the support to separately record blue, green and red exposing radiation. The blue recording emulsion layer unit is typically constructed to provide a yellow dye image on processing, the green recording emulsion layer unit is typically constructed to provide a magenta dye image on processing, and the red recording emulsion layer unit is typically constructed to provide a cyan dye image on processing. Each emulsion layer unit can contain one, two, three or more separate emulsion layers sensitized to the same one of the blue, green and red regions of the spectrum. When more than one emulsion layer is present in the same emulsion layer unit, the emulsion layers typically differ in speed. Typically interlayers containing oxidized developing agent scavengers, such as ballasted hydroquinones or aminophenols, are interposed between the emulsion layer units to avoid color contamination. Ultraviolet absorbers are also commonly coated over the emulsion layer units or in the interlayers. Any convenient conventional sequence of emulsion layer units can be employed, with the following being the most typical:

---

|                                                               |
|---------------------------------------------------------------|
| Surface Overcoat                                              |
| Ultraviolet Absorber                                          |
| Red Recording Cyan Dye Image Forming Emulsion Layer Unit      |
| Scavenger Interlayer                                          |
| Ultraviolet Absorber                                          |
| Green Recording Magenta Dye Image Forming Emulsion Layer Unit |
| Scavenger Interlayer                                          |
| Blue Recording Yellow Dye Image Forming Emulsion Layer Unit   |
| Reflective Support                                            |

---

Further illustrations of this and other layers and layer arrangements in multicolor photographic elements are provided in *Research Disclosure*, Item 36544, cited above, Section XI. Layers and layer arrangements.

Each emulsion layer unit of the multicolor photographic elements contain a dye image forming compound. The dye image can be formed by the selective destruction, formation or physical removal of dyes. Element constructions that form images by the physical removal of preformed dyes are illustrated by *Research Disclosure*, Vol. 308, December 1989, Item 308119, Section VII. Color materials, paragraph H. Element constructions that form images by the destruction of dyes or dye precursors are illustrated by *Research Disclosure*, Item 36544, previously cited, Section X. Dye image formers and modifiers, Subsection A. Silver dye bleach. Dye-forming couplers are illustrated by *Research*

*Disclosure*, Item 36544, previously cited, Section X. Subsection B. Image-dye-forming couplers. It is also contemplated to incorporate in the emulsion layer units dye image modifiers, dye hue modifiers and image dye stabilizers, illustrated by *Research Disclosure*, Item 36544, previously cited, Section X. Subsection C. Image dye modifiers and Subsection D. Hue modifiers/stabilization. The dyes, dye precursors, the above-noted related addenda and solvents (e.g., coupler solvents) can be incorporated in the emulsion layers as dispersions, as illustrated by *Research Disclosure*, Item 36544, previously cited, Section X. Subsection E. Dispersing and dyes and dye precursors.

Materials useful in the preparation of color papers are further illustrated by current commercial practice as, for example, by EDGE™, PORTRA™ or SUPRA™, Color Papers as sold by Eastman Kodak Company, by FUJI™ FA-family Color Papers and FUJI Type D Digital Paper as sold by Fuji Photo Film, by KONICA™ QA-family Color Papers as sold by Konishiroku Industries, by DURATRANS™ and DURACLEAR™ display films as sold by Eastman Kodak Company and by KONSENSUS-II™ display films as sold by Konishiroku Industries. It is also contemplated that the emulsion composition of the invention may be advantageously incorporated into the elements described in an article titled "Typical and Preferred Color Paper, Color Negative, and Color Reversal Photographic Elements and Processing," published in *Research Disclosure*, February 1995, Item 37038. The advantages of the current invention may be achieved by modifying any of these formulations to conform to the requirements set forth in the specification. The exact magnitude of the benefits achieved will, of course, depend on the exact details of the formulations involved but these will be readily apparent to the skilled practitioner.

Silver halide emulsions satisfying the grain requirements described above can be present in any one or combination of the emulsion layer units. Additional useful multicolor, multilayer formats for an element of the invention include Structures I-IV as described in U.S. Pat. No. 5,783,373 referenced above, which is incorporated by reference herein. Each of such structures in accordance with the invention would contain at least one silver halide emulsion comprised of high chloride grains as described above. In accordance with preferred embodiments, at least the blue-sensitized, yellow dye image-forming unit of such elements comprises such a high chloride emulsion. Preferably each of the emulsion layer units contain an emulsion satisfying these criteria.

Conventional features that can be incorporated into multilayer (and particularly multicolor) recording elements contemplated for use in the method of the invention are also illustrated by *Research Disclosure*, Item 38957, cited above:

XI. Layers and layer arrangements

XII. Features applicable only to color negative

XIII. Features applicable only to color positive

B. Color reversal

C. Color positives derived from color negatives

XIV. Scan facilitating features.

In addition to conventional optical exposure printing, recording elements comprising radiation sensitive iodide-banded high chloride emulsions according to this invention can be image-wise exposed in a pixel-by-pixel mode using suitable high energy radiation sources typically employed in electronic printing methods. In a typical electronic printing method, an original image is first scanned to create a digital representation of the original scene. The data obtained is

usually electronically enhanced to achieve desired effects such as increased image sharpness, reduced graininess and color correction. The exposure data is then provided to an electronic printer which reconstructs the data into a photographic print by means of small discrete elements (pixels) that together constitute an image. In a conventional electronic printing method, the recording element is scanned by one or more high energy beams to provide a short duration exposure in a pixel-by-pixel mode using a suitable source such as a cathode ray tube (CRT), light emitting diode (LED) or laser. Such methods are described in the patent literature, including, for example, Hioki U.S. Pat. No. 5,126,235; European Patent Application 479 167 A1 and European Patent Application 502 508 A1. Also, many of the basic principles of electronic printing are provided in Hunt, *The Reproduction of Colour*, Fourth Edition, pages 306-307, (1987).

Once imagewise exposed, the recording elements can be processed in any convenient conventional manner to obtain a viewable image. Such processing is illustrated by *Research Disclosure*, Item 38957, cited above:

XVIII. Chemical development systems

XIX. Development

XX. Desilvering, washing, rinsing and stabilizing

The described elements can be also processed in the ionic separation imaging systems which utilize the sulfonamidonaphthol diffusion transfer technology. Such a photographic product comprises at least one image dye providing element comprising at least one layer of photosensitive silver halide emulsion with which is associated a non-diffusible image dye-providing substance. After image-wise exposure, a coating is treated with an alkaline processing composition in the presence of a silver halide developing agent in such a way that for each dye-image forming element, a silver image is developed. An image-wise distribution of oxidized developer cross-oxidizes the molecule of the image dye-providing compound. This, in an alkaline medium, cleaves to liberate a diffusible image dye. A preferred system of this type is disclosed in Fleckenstein U.S. trial voluntary protest document B351,637, dated Jan. 28, 1975. Other patents include: U.S. Pat. No. 4,450,224 and 4,463,080, and U.K. Patents 2,026,710 and 2,038,041.

In a similar technology, a silver halide photographic process is combined with LED exposure and thermal development/transfer resulting in a high image quality hard copy system incorporating digital exposure technology. Some of the many patents include U.S. Pat. Nos. 4,904,573; 4,952,969; 4,732,846; 4,775,613; 4,439,513; 4,473,631; 4,603,103; 4,500,626; 4,713,319.

The following examples illustrate the practice of this invention. They are not intended to be exhaustive of all possible variations of the invention. Parts and percentages are by weight unless otherwise specified.

EXAMPLES

Example 1

To a reactor incorporating a stirring device disclosed in *Research Disclosure*, Item 38213, and containing 8.756 kg of distilled water, 25 mg of p-glutaramidophenyl disulfide and 251 g of bone gelatin, were added 291 g of 3.8 M sodium chloride salt solution such that the mixture was

15

maintained at a pCl of about 1.05 at approximately 68° C. To this were added 1.9 of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a constant silver nitrate flow rate of about 74 mL/min for about 41 minutes while maintaining pCl constant at about 1.05. Both the silver and sodium salt solution pumps were then turned off and about 0.8 M potassium iodide solution was added to the stirred reaction mixture about 30 seconds at a constant flow rate of about 62.9 mL/min. The resultant iodochloride emulsion was then grown further by conventional controlled double-jet addition for about 3.6 minutes by resumed addition of silver and sodium salt solutions at about 74 mL/min at a pCl of about 1.05. The stirring speed of the stirring device was maintained at 1500 revolutions per minute (RPM) during the entire precipitation process. In addition, cesium pentachloronitrosylsulfonate was added at approximately 4 to 70% into the precipitation, potassium hexacyanoruthenate at 75–80%, and iridium pentachloro-5-methylthiazole was mixed with potassium iodide solution. A silver iodochloride emulsion was thus prepared with 0.2 mole % iodide located at 92% of total grain volume. Cubic edge length was 0.63  $\mu$ m.

A portion of this silver iodochloride emulsion was optimally sensitized by the addition of p-glutaramidophenyl disulfide followed by the addition of a colloidal suspension of aurous sulfide and heat ramped to 60° C. during which time blue sensitizing dye (Dye 1), potassium hexachloroiridate, Lippmann bromide, and 1-(3-acetamidophenyl)-5-mercaptotetrazole were added.

Dye 1

35



## Example 2

To a reactor incorporating a stirring device as disclosed in *Research Disclosure*, Item 38213, and containing 8.756 kg of distilled water, 25 mg of p-glutaramidophenyl disulfide and 251 g of bone gelatin, were added 291 g of 3.8 M sodium chloride salt solution such that the mixture was maintained at a pCl of about 1.05 at approximately 68° C. To this were added 1.9 of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a constant silver nitrate flow rate of about 74 mL/min for about 41 minutes while maintaining pCl constant at about 1.05. Both the silver and sodium salt solution pumps were then turned off and about 0.8 M potassium iodide solution was added to the stirred reaction mixture about 30 seconds at a constant flow rate of about 62.9 mL/min. The resultant iodochloride emulsion was then grown further by

16

pulsed controlled double-jet addition for about 1.2 minutes by resumed addition of silver and sodium salt solutions at about 223 mL/min at a pCl of about 1.05. The stirring speed of the stirring device was maintained at 1500 revolutions per minute (RPM) during the entire precipitation process. In addition, cesium pentachloronitrosylsulfonate was added at approximately 4 to 70% into the precipitation, potassium hexacyanoruthenate at 75–80%, and iridium pentachloro-5-methylthiazole was mixed with potassium iodide solution. A silver iodochloride emulsion was thus prepared with 0.2 mole % iodide located at 92% of total grain volume. Cubic edge length was 0.63  $\mu$ m.

A portion of this silver iodochloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptotetrazole were added.

Blue sensitized emulsions from Example 1 and Example 2 were coated at 19.5 mg silver per square foot and coupler dispersion Y-1 at 50 mg per square foot. The coatings were overcoated with gelatin layer and the entire coating was hardened with bis(vinylsulfonylmethyl)ether.

Y-1



Single layer samples were exposed for 0.1 second to 40 simulate exposure through a color negative film. 0–3.0 density step tablet was used and the source of white light was a Kodak Model 1B sensitometer with a color temperature of 3000° K. and with a combination of the appropriate filters. The exposed coatings were processed using Kodak™ Ektacolor RA-4 processing. Relative log speed was measured at 0.8 absolute density and “toe” value was a density at the point on the photographic curve 0.2 log E faster than a speed point. Minimum density (Dmin) was measured at the region of no exposure.

50

TABLE 1

| Example    | Exterior region (% of total Ag in the grains) | Maximum $R_n$ during the growth of exterior region (min $^{-1}$ ) | Relative Speed |       |       |
|------------|-----------------------------------------------|-------------------------------------------------------------------|----------------|-------|-------|
|            |                                               |                                                                   | Toe Density    | Dmin  |       |
| 1          | 92%–100%                                      | $2.4 \times 10^{-2}$                                              | 100            | 0.350 | 0.070 |
| Comparison |                                               |                                                                   |                |       |       |
| 2          | 92%–100%                                      | $7.2 \times 10^{-2}$                                              | 107            | 0.366 | 0.070 |
| Invention  |                                               |                                                                   |                |       |       |

Softer toe at higher speed and low Dmin was obtained with inventive emulsion.

65 Example 3

Emulsion in this example was precipitated as in Example 1, with the following exceptions: the stirring speed of the

stirring device was maintained at 1575 revolutions per minute (RPM) during the entire precipitation process, 0.2 mole % iodide was located at 90% of total grain volume, iridium pentachloro-5-methylthiazole was located at 92–95 % into the grain growth and resultant edge length was 0.65  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptopotetrazole were added.

#### Example 4

Emulsion in this example was precipitated as in Example 3, with the following exceptions: the stirring speed of the stirring device was maintained at 2925 revolutions per minute (RPM) during the entire precipitation process. Resultant edge length was 0.65  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptopotetrazole were added.

#### Example 5

To a reactor incorporating a stirring device as disclosed in *Research Disclosure*, Item 38213, and containing 8.756 kg of distilled water, 25 mg of p-glutaramidophenyl disulfide and 251 g of bone gelatin, were added 291 g of 3.8 M sodium chloride salt solution such that the mixture was maintained at a pCl of about 1.05 at approximately 68° C. To this were added 1.9 of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a constant silver nitrate flow rate of about 79.7 mL/min for about 1.71 minutes while maintaining pCl constant at about 1.05. Following this nucleation period the rest of silver nitrate and sodium chloride for growth of the 90% of the core grain were delivered with five double-jet pulses at the flow rate of about 232 mL/min separated by hold periods. The duration of the pulses was 0.75, 0.75, 3.0, 5.05, and 3.15 min, respectively. There was a period of rest after each successive pulse. The duration of rests were 5, 3, 3, 3, and 2 min, respectively. Both the silver and sodium salt solution pumps were then turned off and about 0.8 M potassium iodide solution was added to the stirred reaction mixture about 30 seconds at a constant flow rate of about 62.9 mL/min. The resultant iodochloride emulsion was then grown further by pulsed controlled double-jet addition for about 1.35 minutes by resumed addition of silver and sodium salt solutions at about 223 mL/min at a pCl of about 1.05. The solution was then held for one minute. The stirring speed of the stirring device was maintained at 1575 revolutions per minute (RPM) during the entire precipitation process. In addition, cesium pentachloronitrosylsulfate was added at approximately 4 to 70% into the precipitation, potassium hexacyanoruthenate at 75–80%, and iridium pentachloro-5-methylthiazole at 92–95% of the grain volume. A silver iododchloride emulsion was thus prepared with 0.2 mole % iodide located at 90% of total grain volume. Cubic edge length was 0.63  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium

#### Example 6

Emulsion in this example was precipitated as in Example 5, with the following exceptions: the stirring speed of the stirring device was maintained at 2925 revolutions per minute (RPM) during the entire precipitation process. Resultant edge length was 0.63  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptopotetrazole were added.

Blue sensitized emulsions from Example 3 through Example 6 were coated at 19.5 mg silver per square foot and coupler dispersion Y-1 at 50 mg per square foot. The coatings were overcoated with gelatin layer and the entire coating was hardened with bis(vinylsulfonylmethyl)ether.

Single layer samples were exposed for 0.1 second to simulate exposure through a color negative film. 0–3.0 density step tablet was used and the source of white light was a Kodak Model 1B sensitometer with a color temperature of 3000° K. and with a combination of the appropriate filters. The exposed coatings were processed using Kodak™ Ektacolor RA-4 processing. Relative log speed was measured at 0.8 absolute density and “toe” value was a density at the point on the photographic curve 0.2 log E faster than a speed point. Minimum density (Dmin) was measured at the region of no exposure.

TABLE 2

| Reactor stirring effects |                |                                               |                                                                          |                |       |
|--------------------------|----------------|-----------------------------------------------|--------------------------------------------------------------------------|----------------|-------|
| Example                  | Stirring (RPM) | Exterior region (% of total Ag in the grains) | Maximum $R_n$ during the growth of exterior region ( $\text{min}^{-1}$ ) | Relative Speed | Dmin  |
| 3<br>Comparison          | 1575           | 90%–100%                                      | $2.4 \times 10^{-2}$                                                     | 100            | 0.073 |
| 4<br>Comparison          | 2925           | 90%–100%                                      | $2.4 \times 10^{-2}$                                                     | 83.1           | 0.068 |
| 5<br>Invention           | 1575           | 90%–100%                                      | $7.2 \times 10^{-2}$                                                     | 100.3          | 0.078 |
| 6<br>Invention           | 2925           | 90%–100%                                      | $7.2 \times 10^{-2}$                                                     | 96.6           | 0.075 |

Relative speed is less sensitive to stirring speed changes in case of inventive emulsion formulations.

#### Example 7

Emulsion in this example was precipitated similar to that in Example 1, with the following exceptions: 0.2 mole % iodide was located at 91% of total grain volume, iridium pentachloro-5-methylthiazole was located at 92–95 % into the grain, the reagent volumes and flow rates were 10 times larger, and from an initial value of 958 RPM, the stirring speed was varied linearly with the total volume of dispersing medium in the reactor. The resultant cubic edge length was 0.61  $\mu\text{m}$ .

A portion of this silver iododchloride emulsion was optimally sensitized by the addition of p-glutaramidophenyl

disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptotetrazole were added.

5

### Example 8

Emulsion in this example was precipitated similar to that in Example 2, with the following exceptions: 0.2 mole % iodide was located at 91% of total grain volume, iridium pentachloro-5-methylthiazole was located at 92–95 % into the grain, the reagent volumes and flow rates were 10 times larger, and from an initial value of 958 RPM, the stirring speed was varied linearly with the total volume of dispersing medium in the reactor. The resultant cubic edge length was 0.61  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptotetrazole were added.

10

15

20

### Example 9

Emulsion in this example was precipitated similar to that in Example 5, with the following exceptions: 0.2 mole % iodide was located at 91% of total grain volume, iridium pentachloro-5-methylthiazole was located at 92–95 % into the grain, the reagent volumes and flow rates were 10 times larger for the precipitation up to iodide addition. The reactant flow rates after iodide addition were the same as in Example 7. From an initial value of 958 RPM, the stirring speed was varied linearly with the total volume of dispersing medium in the reactor. The resultant cubic edge length was 0.61  $\mu\text{m}$ .

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptotetrazole were added.

30

35

40

45

### Example 10

Emulsion in this example was precipitated similar to that in Example 6, with the following exceptions: 0.2 mole % iodide was located at 91% of total grain volume, iridium pentachloro-5-methylthiazole was located at 92–95 % into the grain, the reagent volumes and flow rates were 10 times larger. From an initial value of 958 RPM, the stirring speed was varied linearly with the total volume of dispersing medium in the reactor. The resultant cubic edge length was 0.61  $\mu\text{m}$ .

50

55

A portion of this silver iododchloride emulsion was optimally sensitized by the addition of p-glutaramidophenyl disulfide followed by the addition of a colloidal suspension of aurous sulfide and heat ramped to 60° C. during which time blue sensitizing dye, Dye 1, potassium hexachloroiridate, Lippmann bromide, and 1-(3-acetamidophenyl)-5-mercaptotetrazole were added.

60

Blue sensitized emulsions from Example 7 through Example 10 were coated as "Yellow emulsion YE1" in the following multialyer format:

| Format 1 |                              |                            |
|----------|------------------------------|----------------------------|
|          | Item Description             | Laydown mg/ft <sup>2</sup> |
| Layer 1  | <u>Blue Sensitive Layer</u>  |                            |
|          | Gelatin                      | 122                        |
|          | Yellow emulsion YE1 (as Ag)  | 19.5                       |
|          | Y-1                          | 45                         |
|          | ST-1                         | 45                         |
|          | S-1                          | 20                         |
| Layer 2  | <u>Interlayer</u>            |                            |
|          | Gelatin                      | 70                         |
|          | SC-1                         | 6                          |
|          | S-1                          | 17                         |
| Layer 3  | <u>Green Sensitive Layer</u> |                            |
|          | Gelatin                      | 117                        |
|          | Magenta emulsion (as Ag)     | 7                          |
|          | M-1                          | 29                         |
|          | S-1                          | 8                          |
|          | S-2                          | 3                          |
|          | ST-2                         | 2                          |
|          | ST-3                         | 17.7                       |
|          | ST-4                         | 57                         |
|          | PMT                          | 0.1                        |
| Layer 4  | <u>UV Interlayer</u>         |                            |
|          | Gelatin                      | 68.4                       |
|          | UV-1                         | 3                          |
|          | UV-2                         | 17                         |
|          | SC-1                         | 5.13                       |
|          | S-1                          | 3                          |
|          | S-3                          | 3                          |
| Layer 5  | <u>Red Sensitive Layer</u>   |                            |
|          | Gelatin                      | 126                        |
|          | Cyan emulsion (as Ag)        | 17                         |
|          | C-1                          | 39                         |
|          | S-1                          | 39                         |
|          | UV-2                         | 25                         |
|          | S-4                          | 3                          |
|          | SC-1                         | 0.3                        |
| Layer 6  | <u>UV Overcoat</u>           |                            |
|          | Gelatin                      | 48                         |
|          | UV-1                         | 2                          |
|          | UV-2                         | 12                         |
|          | SC-1                         | 4                          |
|          | S-1                          | 2                          |
|          | S-3                          | 2                          |
| Layer 7  | <u>SOC</u>                   |                            |
|          | Gelatin                      | 60                         |
|          | SC-1                         | 2                          |
|          | L-1                          | 2                          |

Y-1



ST-1 = N-tert-butylacrylamide / n-butyl acrylate copolymer (50:50)

S-1 = dibutyl phthalate

-continued

Format 1

Item Description

Laydown mg/ft<sup>2</sup>

SC-1



M-1

S-2 = diundecyl phthalate



PMT = 1-phenyl-5-mercaptopurine



S-3 = 1,4-Cyclohexyldimethylene bis(2-ethylhexanoate)

-continued

Format 1

Item Description

Laydown mg/ft<sup>2</sup>

5

C-1



S-4 = 2-(2-Butoxyethoxy)ethyl acetate

20 Each of the multicolor, multilayer coatings was exposed by a 1700 Lux tungsten lamp with a 3000° K. temperature for 0.5 seconds followed by processing in Kodak™ Ektacolor RA-4 processing chemistry in a roller transport processor. Filtration for the red sensitive layer was a Wratten 70, for the green sensitive layer a Wratten 99+0.3 neutral density, and for the blue Wratten 48+2B+0.8 neutral density. Emulsion coating performance was judged by measuring (a) photographic speed in relative Log exposure units at a density of 0.8, (b) a lower scale “toe” density at 0.2 Log E lower exposure than the speed point. The Dmin is a measurement of the density of the processed coating in the area without exposure.

ST-2

25

30

35

40

45

50

TABLE 3

| Example       | Exterior region<br>(% of total Ag<br>in the grains) | Maximum R <sub>n</sub><br>during the<br>growth of ex-<br>terior region<br>(min <sup>-1</sup> ) | Relative<br>Speed | Toe<br>Density | Dmin  |
|---------------|-----------------------------------------------------|------------------------------------------------------------------------------------------------|-------------------|----------------|-------|
| Comparison 7  | 91%-100%                                            | 2.7 × 10 <sup>-2</sup>                                                                         | 100.0             | 0.357          | 0.083 |
| Comparison 8  | 91%-100%                                            | 7.3 × 10 <sup>-2</sup>                                                                         | 102.3             | 0.382          | 0.082 |
| Invention 9   | 91%-100%                                            | 2.7 × 10 <sup>-2</sup>                                                                         | 102.6             | 0.360          | 0.083 |
| Comparison 10 | 91%-100%                                            | 7.3 × 10 <sup>-2</sup>                                                                         | 104.7             | 0.388          | 0.084 |
| Invention     |                                                     |                                                                                                |                   |                |       |

55 Softer toe at higher speed and low Dmin was obtained with inventive emulsions.

## Example 11 (Comparison)

To a reactor incorporating a stirring device as disclosed in *Research Disclosure*, Item 38213, and containing 8.764 Kg of distilled water and 251 g of bone gelatin, were added 291 g of 3.8 M sodium chloride salt solution such that the mixture was maintained at a pH of about 1.05 at approximately 68° C. To this were added 1.9 g of 1,8-dihydroxy-3,6-dithiaoctane approximately 30 seconds before commencing introduction of silver and chloride salt solutions. 60 Aqueous solutions of about 3.7 M silver nitrate and about 3.8 M sodium chloride were then added by conventional controlled double-jet addition at a constant silver nitrate flow rate of about 74 mL/min for about 41 minutes while maintaining pH constant at about 1.05. Both the silver and sodium salt solution pumps were then turned off and about 0.4 M potassium iodide solution was added to the stirred reaction mixture about 3 minutes at a constant flow rate of

about 21 mL/min. The resultant iodochloride emulsion was then grown further by conventional controlled double-jet addition for about 4.5 minutes by resumed addition of silver and sodium salt solutions at about 74 mL/min at a pCl of about 1.05. The stirring speed of stirring device was maintained at 1500 revolutions per minute during the entire precipitation process.

A silver iodochloride cubic grain emulsion was prepared having the characteristics summarized below in Table 4.

Example 12 (Comparison)

Example 11 was repeated, except that the rotation of the stirring device was maintained at 2250 rpm. A silver iodochloride cubic grain emulsion was prepared having the characteristics summarized below in Table 4.

Example 13 (Comparison)

Example 1 was repeated, except that the rotation of the stirring device was maintained at 3000 rpm. A silver iodochloride cubic grain emulsion was prepared having the characteristics summarized below in Table I.

Example 14 (Invention)

To a reactor incorporating a stirring device as disclosed in *Research Disclosure*, Item 38213, and containing 8.764 Kg of distilled water and 251 g of bone gelatin, were added 291 g of 3.8 M sodium chloride salt solution such that the mixture was maintained at a pCl of about 1.05 at approximately 68° C. To this were added 1.9 g of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a constant silver nitrate flow rate of about 82 mL/min for about 1.75 minutes while maintaining pCl constant at about 1.05.

Then the silver nitrate and sodium chloride salt solution were introduced into the reactor simultaneously in sixteen discrete pulses. Each pulse consisted of a constant silver nitrate flow rate of 350 mL/min and a balancing flow rate of sodium chloride solution such that pCl is maintained at approximately 1.05. The following sequence of pulses and intervals were employed:

| event    | minutes |
|----------|---------|
| pulse 1  | 0.5     |
| interval | 10      |
| pulse 2  | 0.5     |
| interval | 5       |
| pulse 3  | 0.5     |
| interval | 5       |
| pulse 4  | 0.33    |
| interval | 2       |
| pulse 5  | 0.33    |
| interval | 2       |
| pulse 6  | 0.33    |
| interval | 2       |
| pulse 7  | 0.33    |
| interval | 2       |
| pulse 8  | 0.33    |
| interval | 2       |
| pulse 9  | 0.33    |
| interval | 2       |
| pulse 10 | 0.7     |
| interval | 2       |

-continued

|    | event    | minutes |
|----|----------|---------|
| 5  | pulse 11 | 0.8     |
|    | interval | 2       |
|    | pulse 12 | 0.8     |
|    | interval | 2       |
|    | pulse 13 | 0.51    |
|    | interval | 2       |
| 10 | pulse 14 | 0.48    |
|    | interval | 2       |
|    | pulse 15 | 0.48    |
|    | interval | 2       |
| 15 | pulse 16 | 0.95    |
|    | interval | 4       |

Both The silver and sodium salt solution pumps were then turned off and about 0.4 M potassium iodide solution was added to the stirred reaction mixture about 3 minutes at a constant flow rate of about 21 mL/min. The resultant iodochloride emulsion was then grown further by the pulse process by way of two additional pulses similar to those described above. The duration of the pulses were 0.5 and 0.48 minute, respectively, and the duration of the interval following the pulse was 2 and 3 minutes, respectively. The stirring speed of the mixing device was maintained at 1750 rpm during the entire precipitation process.

A silver iodochloride cubic grain emulsion was prepared having the characteristics summarized below in Table 4.

Example 15 (Invention)

Example 14 was repeated, except that the rotation of the stirring device was maintained at 2250 rpm. A silver iodochloride cubic grain emulsion was prepared having the characteristics summarized below in Table 4.

Example 16 (Invention)

Example 14 was repeated, except that the rotation of the stirring device was maintained at 2750 rpm. A silver iodochloride cubic grain emulsion was prepared having the characteristics summarized below in Table 4.

TABLE 4

| Example       | Edge Length (μm) | Roundness Coefficient | Stirring (rpm) | Pulsed Flow |
|---------------|------------------|-----------------------|----------------|-------------|
| 11 Comparison | 0.64             | 16.7                  | 1500           | no          |
| 12 Comparison | 0.65             | 10.5                  | 2250           | no          |
| 13 Comparison | 0.65             | 8.7                   | 3000           | no          |
| 14 Invention  | 0.66             | 10                    | 1750           | yes         |
| 15 Invention  | 0.67             | 10                    | 2250           | yes         |
| 16 Invention  | 0.67             | 10                    | 2750           | yes         |

The term "roundness coefficient" hereinafter assigned the symbol "n" is a measure of the degree to which silver halide grain comers are rounded. n is chosen to satisfy the formula:

$$x^n + y^n = R^n$$

where R is any vector extending from the center of a {100} crystal face of a grain to the projected peripheral edge of the grain viewed normal to the {100} crystal face; x is an X axis coordinate of R; y is a Y axis coordinate of R; and X and Y

are mutually perpendicular axes in the plane of the {100} crystal face. For the circle:  $x^2+y^2=R^2$ . Thus, for a circle, the roundness coefficient  $n$  is 2. When the roundness coefficient  $n$  is increased to infinity ( $\infty$ ), a square, is generated. Squares are, of course devoid of roundness. Notice that as the value  $n$  decreases from infinity to 2, the roundness of the peripheral boundary progressively increases. The Roundness Coefficient values in Table 4 indicate that Examples 14-16 demonstrate less dependence upon the manufacturing conditions (in the form of stirring rate), thus demonstrating a more robust process.

It is specifically contemplated that emulsions prepared in accordance with the invention may be sensitized with red, green, and blue sensitizing dyes and be incorporated in a color paper format as described in Example 4 of U.S. Pat. No. 5,783,373, incorporated by reference herein. It is also specifically contemplated to employ emulsions in accordance with the invention in place of the Yellow emulsion YE1 in "Format 1" of the Examples of concurrently filed, copending, commonly assigned U.S. Ser. No. 09/475,839 (Kodak Docket 80208AJA) incorporated by reference above.

The invention has been described in detail with particular reference to preferred embodiments thereof, but it will be understood that variations and modifications can be effected within the spirit and scope of the invention.

What is claimed is:

1. A process for the preparation of a radiation-sensitive silver halide emulsion comprised of high chloride cubical silver halide grains containing from 0.05 to 3 mole percent iodide, based on total silver, where the iodide is incorporated in the grains in a controlled, non-uniform distribution forming a core containing at least 50 percent of total silver, an iodide free surface shell having a thickness of greater than 50 Å, and a sub-surface shell that contains a maximum iodide concentration, the process comprising:

(a) providing in a stirred reaction vessel a dispersing medium and host high chloride silver halide cubical grains comprising a speed enhancing amount of iodide, and

(b) precipitating silver halide onto the host grains by introducing at least a silver salt solution into the dispersing medium at a rate such that the normalized molar addition rate,  $R_n$ , is above  $3.0 \times 10^{-2} \text{ min}^{-1}$ ,  $R_n$  satisfying the formula:

$$R_n = [Q_f \times C_f]/M$$

where

$Q_f$  is the volumetric rate of addition, in L/min, of silver salt solution into the reaction vessel,

$C_f$  is the concentration, in moles/L, of the silver salt solution, and

$M$  is total moles of silver halide in the host grains in the reaction vessel at the precise moment of addition of the silver salt solution.

2. The process according to claim 1, wherein in step (b) a halide salt solution is simultaneously introducing into the dispersing medium with the silver salt solution.

3. The process according to claim 1, wherein only silver salt solution is added during step (b).

4. The process according to claim 1 wherein iodide is incorporated in the host grains by adding an alkali metal iodide salt solution during precipitation of host grains provided in step (a).

5. The process according to claim 1 wherein iodide is incorporated in the host grains by adding silver iodide seed grains during precipitation of host grains provided in step (a).

6. The process according to claim 1 wherein the host grains provided in step (a) are prepared by a precipitation process wherein a silver salt solution is introduced into a dispersing medium in a reaction vessel at a rate such that the normalized molar addition rate,  $R_n$ , is above  $3.0 \times 10^{-2} \text{ min}^{-1}$ .

7. The process according to claim 1 wherein the host grains provided in step (a) are prepared by a precipitation process wherein a silver salt solution is introduced into a dispersing medium in a reaction vessel at a rate such that the normalized molar addition rate,  $R_n$ , is below  $3.0 \times 10^{-2} \text{ min}^{-1}$ .

8. The process according to claim 1 wherein the high chloride cubical silver halide grains contain at least 70 mole percent chloride, based on silver.

9. The process according to claim 1 wherein the high chloride cubical silver halide grains contain at least 90 mole percent chloride, based on silver.

10. A photographic element comprising a support having coated thereon a radiation sensitive emulsion layer comprising a high chloride emulsion prepared according to claim 1.

11. A process for the preparation of a radiation-sensitive silver halide emulsion comprised of high chloride cubical silver halide grains containing from 0.05 to 3 mole percent iodide, based on total silver, where the iodide is incorporated in the grains in a controlled, non-uniform distribution forming a core containing at least 50 percent of total silver, an iodide free surface shell having a thickness of greater than 50 Å, and a sub-surface shell that contains a maximum iodide concentration, the process comprising:

(a) providing in a stirred reaction vessel a dispersing medium and host high chloride silver halide cubical grains comprising a speed enhancing amount of iodide, and

(b) precipitating silver halide onto the host grains by introducing only a silver salt solution into the dispersing medium at a rate such that the normalized molar addition rate,  $R_n$ , is above  $3.0 \times 10^{-2} \text{ min}^{-1}$ ,  $R_n$  satisfying the formula:

$$R_n = [Q_f \times C_f]/M$$

where

$Q_f$  is the volumetric rate of addition, in L/min, of silver salt solution into the reaction vessel,

$C_f$  is the concentration, in moles/L, of the silver salt solution, and

$M$  is total moles of silver halide in the host grains in the reaction vessel at the precise moment of addition of the silver salt solution.

12. The process according to claim 11 wherein iodide is incorporated in the host grains by adding an alkali metal iodide salt solution during precipitation of host grains provided in step (a).

13. The process according to claim 11 wherein iodide is incorporated in the host grains by adding silver iodide seed grains during precipitation of host grains provided in step (a).

14. The process according to claim 11 wherein the host grains provided in step (a) are prepared by a precipitation process wherein a silver salt solution is introduced into a dispersing medium in a reaction vessel at a rate such that the normalized molar addition rate,  $R_n$ , is above  $3.0 \times 10^{-2} \text{ min}^{-1}$ .

15. The process according to claim 11 wherein the host grains provided in step (a) are prepared by a precipitation process wherein a silver salt solution is introduced into a

**27**

dispersing medium in a reaction vessel at a rate such that the normalized molar addition rate,  $R_{n*}$ , is below  $3.0 \times 10^{-2}$   $\text{min}^{-1}$ .

16. The process according to claim 11 wherein the high chloride cubical silver halide grains contain at least 70 mole percent chloride, based on silver. 5

**28**

17. The process according to claim 11 wherein the high chloride cubical silver halide grains contain at least 90 mole percent chloride, based on silver.

\* \* \* \* \*

UNITED STATES PATENT AND TRADEMARK OFFICE  
**CERTIFICATE OF CORRECTION**

PATENT NO. : 6,265,145 B1  
DATED : July 24, 2001  
INVENTOR(S) : Mehta et al.

Page 1 of 1

It is certified that error appears in the above-identified patent and that said Letters Patent is hereby corrected as shown below:

Column 25,  
Line 43, change "3.0" to -- 5.0 --

Signed and Sealed this

Nineteenth Day of July, 2005

A handwritten signature in black ink, appearing to read "Jon W. Dudas". The signature is written in a cursive style with a large, stylized "J" and "W".

JON W. DUDAS  
*Director of the United States Patent and Trademark Office*